

## UNITED STATES PATENT OFFICE

2,293,986

## TREATMENT OF FIBERS, THREADS, AND THE LIKE, DERIVED FROM PROTEIN MATERIALS

Theodoor Koch, Oosterbeek, Netherlands, assignor to American Enka Corporation, Enka, N. C., a corporation of Delaware

No Drawing. Application October 9, 1939, Serial No. 298,715. In Germany November 9, 1938

9 Claims. (Cl. 18—54)

The present invention relates to the manufacture of synthetic filamentous materials and more particularly to the treatment of fibers or threads produced from protein solutions such as casein.

In order to increase the water resistance of protein fibers, it is a common expedient to subject the fibers to formaldehyde baths. However, the fibers so treated are by no means sufficiently resistant to hot aqueous solutions such as dye baths. In a weakly acidic dye bath, which is normally employed for dyeing natural wool, protein fibers will lose weight and assume a rubber-like structure and upon drying stick together and become extremely brittle. Moreover, during the drying period the fibers will shrink as much as 30% or 40% and sometimes even more. It is also known to treat protein fibers with baths containing both formaldehyde and an acid, but then the specific procedure is followed of subsequently, immediately washing the fibers acid-free and finally using a neutral after-hardening bath. In this case, also, the fibers are acted on unfavorably in hot dye baths.

In accordance with the broad invention, it has been determined that casein fibers, having improved physical and chemical characteristics particularly with respect to water resistance, can be produced if, after the normal treatment with a formaldehyde solution, the fibers are subjected to a bath containing an aldehyde and an acid and then prior to washing, are given drying treatments including heating in order to partially or completely dehydrate the fibers.

In conducting the process, baths may be employed to which an acid and an aldehyde per se are added, or compounds may be utilized that subsequently give rise to, or form acids or aldehydes or both. For example, compounds of the type triammonium phosphate  $(\text{NH}_4)_3\text{PO}_4$ , zinc chloride  $\text{ZnCl}_2$  and sodium ethyl sulphate  $\text{C}_2\text{H}_5\text{NaSO}_4$  will give an acid reaction in the bath and on subsequent heating or drying; hexamethylene tetramine  $(\text{CH}_2)_6\text{N}_4$ , aldehyde bisulphite  $\text{CH}_2\text{ONaHSO}_3$  and trioxymethylene  $(\text{CH}_2\text{O})_3$  will produce aldehydes; and chlor methyl alcohol  $\text{CH}_2\text{ClOH}$ , methylene sulphate  $\text{CH}_2\text{SO}_4$  and chloromethoxysulphonyl chloride  $\text{CH}_2\text{ClO.SO.Cl}$  will, on heating, give off formaldehyde as well as acids.

Several different types of acids may be used or produced in order to improve the quality of the finished product, but usually the strong acids such as hydrochloric and sulphuric are preferred. Normally, the acid concentration of the bath is 55

maintained rather high, e.g., a pH of 5 will give noticeable improvements, ranging up to a pH of 2 whereinafter the casein fiber has been treated and dried, it has high resistance to hot acid dye baths. Moreover, the shrinkage is reduced to at least 6%. The invention contemplates using even higher concentrations without damaging the fibers, for example, 10% HCl or  $\text{H}_2\text{SO}_4$ .

In order to obtain the best results, the fibers, after they have been dried in acid condition, are heated to a temperature of approximately 100° C.; alternatively the fibers may be dried in acid condition and thereafter heated in an aldehyde vapor.

15 As previously stated, the resulting components should be acids and aldehydes, and if by using this process or any modifications thereof, the incorrect components are formed, corrective measures must be introduced. Certain materials such as water, in which case they may be dissolved in an inert solvent and the fibers immersed in this solution, and after drying, heated.

During heating, if it is desired to accelerate the dehydration, compounds such as butanol may 25 be used to form azeotropic mixtures; or the materials may be distilled with organic compounds that are immiscible with water, for example toluol.

Compounds which dehydrate or have a tanning 30 effect on the fiber can be used to advantage in the acid, aldehyde bath, in this connection the sulphates of aluminum, chromium and sodium may be employed and aromatic sulphonic acids or condensation products of aromatic sulphonic acids with formaldehyde.

The following examples serve to more fully illustrate the invention:

## Example I

40 Fibers produced from an alkaline casein solution are extruded and spun through an acid coagulating bath and thereupon partially hardened in a neutral or weakly acidic bath containing 45 10% formalin and finally washed and dried. The casein fibers are then immersed for one hour in a bath containing 85 parts of water, 10 parts of formaldehyde and 5 parts of HCl. Upon removal from the said bath the fluid is extracted 50 from the casein fibers by pressing or centrifuging, and dried at a temperature of 50° C. The fibers are again heated for one-half hour at 110° C. and finally washed acid-free and dried. The casein fibers treated in accordance with this procedure, were found to be water-resistant when

dyeing in acid dyes at 95° C. and the shrinkage was reduced below 6%.

*Example II*

Casein fibers hardened in the normal way with formalin are immersed air-dried in a solution which contains 95 parts of butanol and 5 parts of methylene sulphate. After an hour, the fibers are centrifuged and the excess butanol removed by distillation and the fibers then heated for two hours at 100° C. Finally they are washed acid-free, finished and dried. Treated in this manner, the fibers are substantially resistant to thermolysis.

*Example III*

Normally hardened casein fibers are treated with a 5% HCl solution without washing, centrifuged and dried. Thereupon they are exposed in a closed container to the action of dry formaldehyde vapor for a period of one hour at a temperature of 110° C. The fibers are then further treated in accordance with Example 2.

*Example IV*

Casein fibers preliminarily hardened in the usual manner are subjected to treatment for one hour in a bath containing 83 parts of water, 4 parts of anhydrous aluminium sulphate, 5 parts of formaldehyde and 8 parts of concentrated sulphuric acid. After centrifuging, the fibers are dried and heated for one-half hour at 115° C. They are finally washed acid-free and finished. These fibers are completely resistant to thermolysis.

While the invention in its preferred embodiments has been described in connection with casein fibers, it is obvious that it is applicable to various types of synthetic fibers of protein origin.

What is claimed is:

1. A process for increasing the water-resistance of protein fibers and the like, that have been previously hardened in an aldehyde bath in the usual manner which comprises subjecting the fibers to the action of an aldehyde and acid bath and thereupon drying and heating the fibers without previous washing.

2. A process for increasing the water-resistance of protein fibers and the like, that have been previously hardened in an aldehyde bath in the usual manner which comprises immersing

the fibers in a bath containing an aldehyde and acid, and thereupon drying and heating the fibers without previous washing.

3. A process for increasing the water-resistance of protein fibers and the like, that have been previously hardened in an aldehyde bath in the usual manner which comprises immersing the fibers in a bath, which bath contains compounds that will form aldehydes and acids, and thereupon drying and heating the fibers without previous washing.

4. A process according to claim 1 wherein the said bath contains a tanning agent.

5. A process according to claim 1 wherein the heating takes place in a medium containing an aldehyde vapor.

6. A process according to claim 1 wherein the drying and heating takes place in the presence of compounds forming azeotropic mixtures with water, which compounds have a boiling point above 100° C.

7. A process for increasing the water-resistance of fibers obtained from alkaline casein solutions which comprises hardening the fibers with a formaldehyde solution, washing and drying, subjecting the fibers to a formaldehyde bath that has an acid concentration between pH 5 and pH 2, extracting the liquid and drying for a time at a temperature approximately 50° C. and 30 then heating for about one-half hour at 110° C., and finally washing the fibers acid-free and drying.

8. A process for increasing the water-resistance of fibers produced from alkaline casein solutions which comprises preliminarily hardening the fibers in a formalin bath, treating the fibers for at least an hour in an aqueous bath containing aluminum sulphate, formaldehyde and sulphuric acid, subjecting the fibers to a two-stage drying operation, the second stage being conducted at a temperature above 100° C., finally washing the fibers acid-free and drying.

9. A process for increasing the water resistance of protein fibers and the like, that have 45 been previously hardened in an aldehyde bath in the usual manner which comprises immersing the fibers in a bath containing substances of the class consisting of aldehydes and acids, and compounds that form aldehydes and acids, and thereupon drying and heating the fibers without previously washing.

THEODOOR KOCH.